# EUROPEAN PATENT SPECIFICATION

(11) **EP 0 157 634 B1**
(45) Date of publication and mention of the grant of the patent: **17.08.1988**
(21) Application number: 85302311.7
(22) Date of filing: 02.04.1985
(51) Int. Cl.: H01J 1/28, H01J 1/14, H01J 9/04

(54) **Tungsten-iridium impregnated cathode**
Wolfram und Iridium enthaltende Vorratskathode
Cathode à réserve contenant du tungstène et de l'iridium

(30) Priority: 02.04.1984 US 595789
(43) Date of publication of application: 09.10.1985
(73) Proprietor: VARIAN ASSOCIATES, INC., Palo Alto, CA 94303 (US)
(72) Inventor: Green, Michael Curzon, Palo Alto California (US)
(74) Representative: Cline, Roger Ledlie

(56) References cited:
- EP-A- 0 028 954
- DE-A- 2 909 958
- US-A- 4 165 473

## Description

### Field of the invention

The invention pertains to thermionic cathodes in which a porous body of refractory metal is impregnated with a molten oxide containing an alkali- earth.

### Prior art

Early impregnated cathodes were made by sintering a body of powdered tungsten to form a porous block. The porous material was impregnated with molten copper or an organic polymerto make it machinable to its desired shape. After machining this impregnant was removed and the porous cathode was impregnated with a molten barium aluminate. U.S. Patent No. 2,700,000 issued January 18,1955 to R. Levi describes such a cathode.

U.S. Patent No. 3,373,307 issued November 12, 1964 describes an improved impregnated cathode in which the emissive surface is coated with iridium or other metals of its group. The coating improves the electron emission, but it has been found that the improvement is often short-lived. A principal problem seems to be that, in an electron tube where high current density is drawn from the cathode at high voltage, ions are formed from the residual gas. They are accelerated back to the cathode and sputter away a thin layer from its surface, removing the iridium.

U.S. Patent No. 4,165,473 issued August 21,1979 to Louis R. Falce and assigned to the assignee of the present invention, discloses a cathode in which particles of iridium orthe like are dispersed among the tungsten particles of the matrix. During sintering the iridium partially alloys with the tungsten. This dispersed cathode solved the problem of surface sputtering. It has been found, however, that the sintering is a very delicate process. If the time and temperature are enough to get a lot of alloying, the emission is often poor. if the sintering is held to a minimum, the emission is initially good, but interdiffusion of iridium and tungsten occurs at operating temperature to form unreactive alloy. This in turn causes the barium supply to the surface to fall off with a resultant decay in emission. Also, shrinkage of the cathode button can take place with the distortion of the emitting surface, which impacts adversely on the electron optics of the gun.

### Purpose of the invention

An object of the invention is to provide a cathode with improved emission over a long life span.

Another object is to provide a cathode which is tolerant of the exact parameters of manufacture and operation.

These objects are realized in accordance with the invention, which provides thermionic cathode comprising:
a porous matrix of particles of an alloy of (a) at least one noble metal of the platinum group and (b) at least one refractory metal selected from tungsten and molybdenum,
porous agglomerates composed of one of said refractory metals and dispersed in said matrix, the porous agglomerates being so large as compared with said particles of the alloy that alloying with the noble metal is prevented except on the outer surface of the agglomerates, and
the pores of said matrix and said agglomerates being filled with an active material comprising at least one alkaline earth oxide.

### Brief description of the drawings

Fig. 1 is a schematic enlarged cross-section of a portion of a cathode embodying the invention.
Fig. 2 is a cross section of a concave cathode for a linear-beam microwave tube.

### Description of the preferred embodiments

As a basis for the physical form of our inventive cathode, following is a brief description of our concept of the operation of a dispenser cathode. Basically there are two requirements which in prior-art cathodes were often at odds.

First, an emitting surface is required which has a low work-function. This is provided by a thin (sometimes monatomic) layer of an alkaline earth metal such as barium, strontium, calcium or mixtures thereof and often containing oxygen as well.

The second requirement is a means for replenishing the active layer as it is removed in operation by evaporation or sputtering.

In the following description we use the word "tungsten" to include molybdenum. We use the word "barium" as an example of an alkaline earth metal, which may additionally include calcium, strontium, and alloys thereof as well.

In the original tungsten matrix cathodes the emitting layer is on the surface of the porous tungsten. It has a moderately low work function and thus give emission capability of a few amperes per square centimeter. The life is very good however, because the surfaces of the tungsten matrix in contact with the barium aluminate impregnant are chemically reducing at the operating temperature of around 1000°C, sufficient to react with the oxide and product free barium atoms. This barium can then be transported to the active surface to re-activate it as fast as surface material was removed.

The addition of a surface layer of iridium or other metals of the platinum group produces a significant further lowering of the work function and hence higher emission density. The work function is believed to be affected by the extentto which the surface metal can polarize the barium rlipole layer.

The iridium provides tighter bonding of the barium atoms, reducing evaporation as well as work function. Iridium, however, has low reducing power. When it is added to the matrix as taught by U.S. Patent No. 4,165,473 it alloys with the tungsten, perhaps more as a surface coating than a bulk alloy. This will decrease the reducing power of the tungsten and slow the replenishment of lost barium.

In carrying out this invention as shown in Figure 1, we provide relatively large, porous "islands" 14 of pure tungsten in a matrix 10 of tungsten- iridium alloy particles 12. The iridium provides a surface 20 which can be activated to have a low work function. Even when surface material is removed, the surface is regenerated. The pure tungsten islands are porous grains, each formed from many fine tungsten particles 16 sintered together. Their large surface area provides a reducing interface with the impregnant 18 to produce an adequate supply of reactivating barium to the emitting surface. Their size and convolutions are sufficient to prevent alloying with the iridium except on their outer surfaces.

As an example of the process for producing the inventive cathode, the following steps are performed:
1. Porous tungsten bar stock is made by compressing and sintering fine tungsten powder particles of about 5 microns diameter, as is well known in the art. The density of the resulting bar is about 72% of that of solid tungsten.
2. The bar is impregnated with a liquid plastic monomer such as methyl methacrylate which is then polymerized by heat as described in U.S. Patent No. 3,076,916 issued February 5, 1963 to Otto G. Koppius. The bar is broken down into a mixture of agglomerates by machining, such as turning on a lathe.
3. The plastic infiltrant is removed from the agglomerates and any carbon residues are cleaned up by firing in wet hydrogen at 750°C.
4. Agglomerates larger than 150 microns are sieved out and discarded.
5. The tungsten agglomerates and fines which pass through a 100 mesh sieve are tumble mixed with -325 mesh iridium powder in the proportion of 60 parts by weight of tungsten to 40 parts of iridium.
6. The power mix is pressed at 3.4x10⁵ N/m² and the resultant compact sintered in hydrogen at 1720°C to give pure tungsten agglomerates dispersed in a matrix of iridium-tungsten alloy. Most of the agglomerates are large compared to the iridium particles. The tungsten fines alloy with the iridium particles.
7. The sintered body is then manufactured into cathode elements by conventional techniques:
   7a. Molten copper is infiltrated into the pores to provide support for machining.
   7b. The cathode shapes are machined from the copper-infiltrated bar.
   7c. The copper is removed by chemical etching and hydrogen firing.
   7d. The cathode elements are impregnated in hydrogen or vacuum with barium-calcium aluminate, typically 6BaO:1CaO:2Al₂O₃.
8. The emissive surface may be sputter coated with a codeposited 50:50 mixture of tungsten and iridium. This coating is nearly the same composition as the iridium-tungsten alloy mixture, so its removal by ion sputtering does not seriously affect the cathode.

This embodiment of the invention has been found to provide emission current densities equal or superior to, and lives exceeding those of, the best examples of the prior art. However, unlike the prior art, this cathode can be reproducibly manufactured. Cathodes capable of 8 amperes per square centimeter below 1050°C brightness have been produced with greater than 90% yield. Running temperatures for a given current density were within 10°C of each other. The performance was very stable with operating time. Cathodes have passed 4,000 hours at 8 Alcm² with practically no change.

The large agglomerates alloy with the iridium during sintering and subsequent operation, but due to their size the alloying occurs only at their outer surfaces. They are porous and are completely infiltrated by the active oxide so that the reduction to produce barium goes on freely in their interior.

Fig. 2 illustrates the incorporation of the emitting element (the "cathode" proper) in a cathode structure as used in a linear-beam microwave tube. Cathode 10' is machined to have a smooth concave emitting surface 20' (usually spherical). Its base is fitted onto a cylindrical support 22, as of molybdenum or tantalum and attached thereto as by welding at junction 23. A radiant heater 24, as of tungsten wire in a bifilar spiral is supported by its legs 25 by the support means (not shown) of cylinder 22.

It will be obvious to those skilled in the art that many variations of the above-described cathode and process of production can be made within the true scope of the invention as claimed. The proportions of the various components can cover a wide range. For example, we believe the ratio of iridium to tungsten may vary from about 20% to about 80%. The "barium" may also include calcium, and/or strontium, or mixtures thereof. The "tungsten" may be molybdenum, tungsten, or their alloys. The "iridium" may be osmium, ruthenium, rhenium, iridium or alloys thereof.

## Claims

1. A thermionic cathode (10') comprising:
a porous matrix (10) of particles (12) of an alloy of (a) at least one noble metal of the platinum group and (b) at least one refractory metal selected from tungsten and molybdenum,
porous agglomerates (14) composed of one of said refractory metals and dispersed in said matrix, the porous agglomerates being so large as compared with said particles of the alloy that alloying with the noble metal is prevented except on the outer surface of the agglomerates, and
the pores of said matrix and said agglomerates being filled with an active material (18) comprising at least one alkaline earth oxide.

2. The cathode (10') of claim 1, wherein said active material further comprises aluminum oxide.

3. The cathode (10') of claim 1 or 2, wherein said platinum group metal is iridium.

4. The cathode (10') of any preceding claim wherein said refractory metal is tungsten.

5. The cathode (10') of any preceding claim, further comprising a smooth surface (20') adapted for electron emission.

6. The cathode (10') of claim 5, further comprising a uniform, homogeneous layer on said smooth surface, said layer comprising said metal of the platinum group and said refractory metal.

7. The cathode (10') of claim 6, wherein the composition of said layer is approximately the average composition of said matrix.

8. The cathode (10') of any preceding claim, further comprising means (22) for supporting said cathode.

9. The cathode (10') of any preceding claim, further comprising means (24) for heating said cathode to a temperature of about 1000°C to 1100°C.

10. A process for manufacturing a thermionic cathode (10') comprising the steps of:
forming a porous body by sintering together particles of at least one refractory metal selected from tungsten and molybdenum,
mechanically breaking down said porous body into fines and agglomerates (14) of the refractory metal,
mixing said fines and agglomerates (14) with particles (12) containing at least one noble metal selected from iridium, rhenium, ruthenium and osmium, which particles are so small as compared with said agglomerates, that alloying with the noble metal takes place only on the outer surface of the agglomerates and with the fines,
compressing said mixture,
sintering said mixture to adhere said particles and said agglomerates into a porous mass (10),
impregnating said mass with a molten oxide (18) comprising an alkaline earth oxide.

11. The process of claim 10, further comprising the steps, after sintering said mixture, of:
impregnating said porous mass with a liquid,
converting said liquid to a solid to support said porous mass,
machining said mass to the shape of a desired cathode,
removing said solid.

12. The process of claim 11, further comprising the steps of:
machining on said cathode shape a smooth surface (20') adapted for electron emission,
depositing on said smooth surface a uniform, homogeneous layer comprising said noble metal and said refractory metal.

13. The process of claim 12, wherein the composition of said layer is approximately the average composition of said particles containing said noble metal.

14. The process of any of claims 11 to 13, further comprising the step of affixing said cathode (10) to support means (22).

15. The process of claim 14, further comprising the step of attaching to said support means a heater (24) near said cathode (10) capable of heating said cathode to about 1000 to 1100 degrees Celsius.

## Patentansprüche

1. Glühkathode (10'), die folgendes umfasst:
eine poröse Grundmasse (10) aus Teilchen (12) einer Legierung aus (a) mindestens einem Edelmetall der Platingruppe und (b) mindestens einem hochschmelzenden Metall, das aus Wolfram und Molybdän ausgewählt wird,
poröse Agglomeraten (13), die aus einem der besagten, hochschmelzenden Metalle zusammengestellt werden, die in besagter Grundmasse dispergiert werden, wobei die porösen Agglomerate so gross sind wie vergleichsweise die besagten Teilchen der Legierung, sodass Legierung mit dem Edelmetall ausser auf der äusseren Fläche der Agglomerate verhindert wird, und
die Poren der besagten Grundmasse und der besagten Agglomerate mit einem aktiven Material (18) gefüllt werden, das mindestens ein alkalines Erdoxid enthält.

2. Kathode (10') nach Anspruch 1, bei der besagtes aktives Material ferner Aluminiumoxid enthält.

3. Kathode (10') nach Anspruch 1 oder 2, bei der besagtes Metall der Platingruppe Iridium ist.

4. Kathode (10') nach einem der vorangehenden Ansprüche, bei der das hochschmelzende Metall Wolfram ist.

5. Kathode (10') nach einem der vorangehenden Ansprüche, die ferner eine glatte Oberfläche (20') umfasst, die zur Elektronenemission angepasst ist.

6. Kathode (10') nach Anspruch 5, die ferner eine ebenmässige, homogene Schicht aus besagter glatter Oberfläche umfasst, wobei besagte Schicht besagtes Metall der Platingruppe und besagtes hochschmelzendes Metall umfasst.

7. Kathode (10') nach Anspruch 6, bei der die Zusammensetzung der besagten Schicht ungefähr der durchschnittlichen Zusammensetzung der Grundmasse entspricht.

8. Kathode (10') nach einem der vorangehenden Ansprüche, die ferner Mittel (22) zum Stützen der besagten Kathode umfasst.

9. Kathode (10') nach einem der vorangehenden Ansprüche, die ferner Mittel (24) zum Heizen der besagten Kathode auf eine Temperatur zwischen ungefähr 1000°C und 1100°C umfasst.

10. Verfahren zur Herstellung einer Glühkathode (10'), das folgende Stufen umfasst:
Bildung eines porösen Körpers durch Zusammensintern von mindestens einem hochschmelzenden Metall, das aus Wolfram und Molybdän ausgewählt wird,
mechanisches Zerlegen des besagten, porösen Körpers in Feinanteile und Agglomerate (14) des hochschmelzenden Metalls,
Mischen der besagten Feinanteils und Agglomerate (14) mit Teilchen (12), die mindestens ein Edelmetall enthalten, das aus Iridium, Rhenium, Ruthenium und Osmium ausgewählt wird, deren Teilchen im Vergleich zu besagten Agglomeraten so klein sind, dass das Legieren mit dem Edelmetall nur an der äusseren Oberfläche der Agglomerate und mit den Feinanteilen stattfindet,
Kompression besagter Mischung,
Zusammensintern besagter Mischung, um besagte Teilchen und besagte Agglomerate in einer porösen Masse (10) zu binden,
Impregnieren besagter Masse mit einem geschmolzenen Oxid (18), der ein alkalines Erdoxid enthält.

11. Verfahren nach Anspruch 10, das ferner nach dem Sintern der besagten Mischung die folgenden Stufen umfasst:
Impregnieren der besagten, porösen Masse mit einer Flüssigkeit,
Umwandeln besagter Flüssigkeit in einen Feststoff, um besagte, poröse Masse zu stützen, Formen der besagten Masse in die Form der gewünschten Kathode,
Entnahme des Feststoffes.

12. Verfahren nach Anspruch 11, das ferner folgende Stufen umfasst:
Formen einer glatten zur Elektronenemission angepassten Oberfläche (20') auf besagter Kathodenform,
Ablagern auf besagter, glatten Oberfläche einer ebenmässigen, homogenen Schicht, die besagtes Edelmetall und besagtes hochschmelzendes Metall umfasst.

13. Verfahren nach Anspruch 12, bei dem die Zusammensetzung der besagten Schicht ungefähr der durchschnittlichen Zusammensetzung der besagten, das Edelmetall enthaltenden Teilchen entspricht.

14. Verfahren nach einem der vorangehenden Ansprüche 11 bis 13, das ferner die Stufe des Befestigens der besagten Kathode.(10) auf die Stützmittel (22) umfasst.

15. Verfahren nach Anspruch 14, das ferner die Stufe des Anbringens eines Heizers (24) an besagte Stützmittel in der Nähe der besagten Kathode (10) umfasst, wobei er in der Lage ist, besagte Kathode auf ungefähr 1000 bis 1100 Grad Celsius aufzuheizen.

## Revendications

1. Cathode thermoionique (10') comprenant: une matrice poreuse (10) de particules (12) d'un alliage contenant (a) au moins un métal précieux du groupe du platine et (b) au moins un métal réfractaire choisi parmi le tungstène et le molybdène,
des agglomérés poreux (14) composé de l'un desdits métaux réfractaires et dispersés dans ladite matrice, les agglomérés poreux possédant des dimensions suffisamment importantes par rapport à celles desdites particules de l'alliage, pour que l'alliage avec le métal précieux soit empêché hormis sur la surface extérieure des agglomérés, et
les pores de ladite matrice et desdits agglomérés étant remplis par un matériau actif (18) comprenant au moins un oxyde alcalino-terreux.

2. Cathode (10') selon la revendication 1, dans laquelle ledit matériau actif comporte en outre de l'oxyde d'aluminium.

3. Cathode (10') selon la revendication 1 ou 2, dans laquelle ledit métal du groupe du platine est l'iridium.

4. Cathode (10') selon l'une quelconque des revendications précédentes, dans laquelle ledit métal réfractaire est du tungstène.

5. Cathode (10') selon l'une quelconque des revendications précédentes, comportant en outre une surface lisse (20') adaptée pour réaliser l'émission d'électrons.

6. Cathode (10') selon la revendication 5, comportant en outre une couche homogène et uniforme située sur ladite surface lisse, ladite couche comprenant ledit métal du groupe du platine et ledit métal réfractaire.

7. Cathode (10') selon la revendication 6, dans laquelle la composition de ladite couche est approximativement la composition moyenne de ladite matrice.

8. Cathode (10') selon l'une quelconque des revendications précédentes, comportant en outre des moyens (22) pour supporter ladite cathode.

9. Cathode (10') selon l'une quelconque des revendications précédentes, comportant en outre des moyens (24) pour chauffer ladite cathode à une température d'environ 1000°C à 1100°C.

10. Procédé pour fabriquer une cathode thermoionique (10'), incluant les étapes consistant à:
former un corps poreux par réunion par frittage de particules d'au moins un métal réfractaire choisi parmi le tungstène et le molybdène,
broyer mécaniquement ledit corps poreux sous la forme de fines et d'agglomérés (14) du métal réfractaire,
mélanger lesdites fines et lesdits agglomérés (14) à des particules (12) contenant au moins un métal précieux choisi parmi l'iridium, le rhénium, le ruthénium et l'osmium, ces particules étant suffisamment petites par rapport auxdits agglomérés qu'une liaison par alliage au métal précieux s'effectue uniquement sur la surface extérieure des agglomérés et avec les fines,
comprimer ledit mélange,
fritter ledit mélange pour faire adhérer lesdites particules et desdits agglomérés sous la forme d'une masse poreuse (10),
imprégner ladite masse avec un oxyde fondu (18) comprenant un oxyde alcalino-terreux.

11. Procédé selon la revendication 10, comprenant en outre, après le frittage dudit mélange, les étapes consistant à:
imprégner ladite masse poreuse avec un liquide,
convertir ledit liquide en un solide pour qu'il supporte ladite masse poreuse,
usiner ladite masse pour lui donner la forme d'une cathode désirée,
éliminer ledit solide.

12. Procédé selon la revendication 11, comprenant en outre les étapes consistant à:
former par usinage, dans ladite forme de cathode, une surface lisse (20') adaptée pour réaliser l'émission d'électrons,
déposer sur ladite surface lisse une couche uniforme et homogène comprenant ledit métal précieux et ledit métal réfractaire.

13. Procédé selon la revendication 12, selon lequel la composition de ladite couche est approximativement la composition moyenne desdites particules contenant ledit métal précieux.

14. Procédé selon l'une quelconque des revendications 11 à 13, comprenant en outre l'étape consistant à fixer ladite cathode (10) aux moyens de support (22).

15. Procédé selon la revendication 14, comprenant en outre l'étape consistant à fixer auxdits moyens de support, à proximité de ladite cathode (10), un dispositif de chauffage (24) apte à chauffer ladite cathode à environ 1000 à 1100 degrés Celsius.
